

Nov. 27, 1928.

1,692,818

G. W. CHRISTOPH

METHOD OF SOLDERING RADIATORS

Filed Oct. 2, 1926

Fig. 1.



Fig. 2.



Fig. 3.



Fig. 4.



Fig. 5.



INVENTOR  
George W. Christoph  
by  
Arthur B. Jenkins,  
ATTORNEY.

## UNITED STATES PATENT OFFICE.

GEORGE W. CHRISTOPH, OF WAREHOUSE POINT, CONNECTICUT.

## METHOD OF SOLDERING RADIATORS.

Application filed October 2, 1926. Serial No. 139,096.

My invention relates to a method for constructing devices which are employed for changing the temperatures in liquids, and which may be especially designed for lowering the temperature or cooling the liquid used for preventing overheating in internal combustion engines, and an object of my invention, among others, is the production of a method for making devices of this class, as a 10 radiator, that shall be simple in construction and particularly efficient in operation.

A method embodying my invention and in the practice of which the objects herein set out, as well as others, may be attained, is illustrated in the accompanying drawings, in which—

Figure 1 is a view of a fragment of a radiator showing the parts assembled preliminary to the step of securing them together.

Figure 2 illustrates a vat containing a material for securing the radiator parts together, and in which the radiator is dipped for this purpose.

Figure 3 is a view similar to Figure 1 and showing the parts after treatment in the vat shown in Figure 2.

Figure 4 is a view illustrating an electro-plating apparatus by means of which the outer coating is removed from the radiator.

Figure 5 is a view similar to Figure 1, but illustrating the appearance of the radiator parts after treatment in the device shown in Figure 4.

In the construction of devices for changing the temperature of liquids, and especially in the formation of radiators and like structures employed in automobile construction, as is well known, copper is a metal possessing a high degree of conductivity, but the use of such a metal has heretofore been limited, owing to the difficulty in securing radiating elements composed of copper in place, and in some cases where copper has been used the advantageous features of this conductivity have been much lessened from the fact that the conducting plates have been covered with other metal used to secure the plates in position.

By the use of my invention illustrated and described herein, I have provided means whereby conducting elements composed of copper may be secured in place, as to tubes for conducting liquid, in a very simple and expeditious manner and in such way that the surfaces exposed to the action of air currents shall be of copper, or other proper material.

Such a structure is illustrated in the drawings herein where the numeral 5 indicates a portion of a radiator, as of an automobile, that may be attached to and connected up with an explosive engine in any ordinary and well known manner. The radiator shown, as to its principal parts, is of well known construction embodying tubes 6 extending from the reservoir 7 at the top of the radiator to a chamber 8 at the bottom of the radiator. These tubes pass through plates 9 that are rigidly secured to the tubes in the manner now to be described.

Each of the plates 9 is provided with openings 10 through which the tubes 6 extend, and these openings are preferably provided with flanges 11 to closely fit the tubes.

In practicing my invention a tube and plate structure is formed by assembling the necessary number of tubes and plates in their proper relative positions, and while maintaining said members in such positions in any desirable way the structure is dipped in a molten bath 20 of any material suitable for securing the tubes and plates together, said material being contained in a vat 21. This treatment, when the soldering material cools, will securely fasten the plates to the tubes, it being understood that the plates and tubes, either or both, are composed of metal. The treatment above described, however, will coat the plates and tubes with the soldering material, and it is my purpose, therefore, to remove this material so that the copper surfaces of the tubes and plates shall be exposed.

In securing or soldering the plates and tubes together tin in a molten state may be employed and after the treatment just described it will be found that this material has entered the spaces, as at 12, between the tubes and plates.

The coating 13 of tin or other material may be removed in any suitable manner, it being possible to accomplish this purpose in different ways, but I have found that this coating 100 may be removed or stripped off in a ready manner by employing an electroplating apparatus in which the radiator is placed in an electrolyte 14 contained in a tank 15, the radiator constituting the anode to which the positive wire 16 of an electric circuit is connected. A cathode 17 is suitably arranged in the electrolyte to receive the deposit of tin from the radiator or anode, the cathode being connected with the negative wire 18 in such electric circuit.

After the coating 13 has been removed in the manner above described, or by any other suitable means, it will be found that deposits 19 are retained in the joints between the 5 plates and tubes, thereby securely fastening said parts together, and the copper tubes and plates are left in their original condition with the entire outer surface of the structure constituted of copper and without any coating 10 of other material.

While copper has been mentioned herein as a material of which the tubes and plates are composed, and while tin has been mentioned as a material for soldering or securing the 15 parts together, it will be understood that the invention is not limited to any particular kind of materials for these purposes, but that any suitable material may be employed in the tubes and plate structures, and any suitable 20 material may be employed for soldering or securing the radiator members together.

In accordance with the provisions of the patent statutes I have described the principles of operation of my invention, together 25 with the device which I now consider to represent the best embodiment thereof, but I desire to have it understood that the device shown is only illustrative and that the invention may be carried out by other means 30 and applied to uses other than those above set out.

I claim—

1. The process of securing members together which consists in assembling said 35 members leaving pockets at the joints therebetween, applying a coating to the outer surfaces of said members and simultaneously filling the pockets with the coating material, and then removing the coating material until the 40 surfaces of the members with the exception of said pockets are free of the material.

2. The process of securing members together which consists in assembling said members leaving pockets at the joints there- 45 between, filling said pockets and coating said members by dipping the assembly in a bath of fused metal, and then removing the coating material until the surfaces of the members with the exception of said pockets are 50 free of the material.

3. The process of securing members together which consists in assembling said members leaving pockets at the joints there- 55 between, applying a coating to the outer surfaces of said members and simultaneously filling said pockets to produce an excessive

deposit at the joints, and then placing the assembly in an electrolyte through which an electric current is passed to uniformly remove the coating material until the surfaces 60 of the members with the exception of said pockets are free of the material.

4. The process of securing members together which consists in assembling said members in final relative positions and leaving pockets at the joints therebetween, filling said pockets and uniformly coating said members by dipping the assembly in a bath of fused metal, and then placing the assembly in an electrolyte through which an electric 70 current is passed to uniformly remove the coating material until the surfaces of the members with the exception of said pockets are freed of the material.

5. The process of securing members together which consists in assembling said members and leaving pockets at the joints therebetween, applying a coating of molten metal to the outer surfaces of the members and simultaneously filling said pockets to produce an excessive deposit at the joints, permitting said metal to harden, and then stripping the hardened metal to a uniform depth from all exposed surfaces of the members until the surfaces with the exception of the 80 pockets are freed of the deposited metal.

6. The process of securing members together which consists in assembling said members in their final relative positions leaving pockets at the joints therebetween, dipping said assembly in a bath of molten metal to uniformly coat the exposed surfaces with the exception of the joints where an excessive deposit is made due to said pockets, and then removing the deposited metal by continuing 85 to uniformly strip the same from all exposed surfaces of the assembly until the metal deposited within said pockets is exposed when the stripping action is stopped.

7. The process of securing members together which consists in assembling said members to create joints therebetween, coating said members by dipping the assembly in a bath of fused metal thereby depositing an excess quantity and thickness of metal in the angle at said joints, permitting said deposited metal to harden, and then stripping the hardened metal to a substantially uniform depth over all exposed surfaces until the surfaces of the members are bared except in the angle 100 at said joints.

GEORGE W. CHRISTOPH.